

# UNITED STATES PATENT OFFICE.

HOMER T. YARYAN, OF TOLEDO, OHIO.

## PROCESS OF CONCENTRATING METALLIC ORES BY FLOTATION.

1,191,053.

Specification of Letters Patent.

Patented July 11, 1916.

No Drawing.

Application filed March 29, 1916. Serial No. 87,659.

*To all whom it may concern:*

Be it known that I, HOMER T. YARYAN, a citizen of the United States, residing at Toledo, in the county of Lucas and State of Ohio, have invented a certain new and useful Process of Concentrating Metallic Ores by Flotation; and I do declare the following to be a full, clear, and exact description of the invention, such as will enable others skilled in the art to which it appertains to use the same.

My invention relates to the process of concentrating metallic ores by what is known as "The oil flotation process."

When ores of low grade, such as galena or copper ore, are finely ground and mixed with from three to four parts of water and violently agitated with a small percentage of certain oils, there is formed a stiff froth which seizes upon and carries the metallic particles, which are thus separated from the quartz and other non-metallic particles. The froth with its metallic particles floats to the surface and is allowed to flow off or is removed, carrying with it the concentrate and leaving the gangue which does not attach itself to the froth. The wet concentrate is dried and is now ready for further treatment by the proper metallurgical process. This flotation process is well understood and need not be here more particularly described.

The efficiency of the oil or mixture used in this process is in proportion to the amount required to produce a froth of the necessary amount and consistency for the collection of the ore particles.

There have been employed or proposed, among other agencies, for producing the froth and flotation indicated, coal and pine 40 tars; crude and refined creosote; eucalyptus oil; pine oil; cotton seed oil; petroleum and its products; rosin-oil, and various mixtures of the same, with varying results. These several agents are included in my use herein 45 of the term "oil."

The object of my invention is to greatly increase the amount and permanency of the froth obtainable from these and other oils when agitated with water and ores, and to thereby reduce the quantity and cost of the oil requisite for the treatment of a given quantity of ore; to lessen the time required

for the process, and to increase the percentage of metallic particles extracted. I attain these results by adding to the oil employed 55 the necessary percentage of a resinate of an alkaline metal, such as soda, potash or lime. As a chemical equivalent of these alkaline metals, ammonia may be substituted and combined with rosin to form resinate of 60 ammonia.

In practice, by way of illustration, I obtain a superior "flotation oil" by mixing together fifty per cent. petroleum, fifteen per cent. pine oil and thirty-five per cent. resinate of soda or resinate of ammonia.

It will be understood that rosin oil may be substituted for rosin in the preparation of the resinates above referred to.

The proportions here given, while entirely 70 satisfactory in practice, may, of course, be varied, as conditions may require, without departing from the spirit of my invention.

Having described my invention, what I claim and desire to secure by Letters Patent, 75 is—

1. The process of concentrating metallic ores which consists in agitating the ores in comminuted form in a mixture of water, oil and a suitable resinate, and then, by flotation, recovering the froth thus produced together with its accompanying metallic particles.

2. In the concentration of metallic ores by flotation, the step which consists in agitating 85 the ores in a mixture of water, oil and a resinate of an alkaline metal.

3. The process of concentrating metallic ores which consists in agitating the ores in comminuted form in water to which is added 90 a mixture consisting of sixty-five per cent. oil and thirty-five per cent. resinate of soda, — petroleum constituting upward of fifty per cent. of the whole, — and then by flotation recovering the froth thus produced 95 together with its accompanying metallic particles.

In testimony whereof I affix my signature in presence of two witnesses.

HOMER T. YARYAN.

Witnesses:

GERTRUDE BRACKER,  
ALMON HALL.